

Patented May 1, 1923.

1,453,976

# UNITED STATES PATENT OFFICE.

BENNETT GROTTA, OF TAMAQUA, PENNSYLVANIA, ASSIGNOR TO ATLAS POWDER COMPANY, OF WILMINGTON, DELAWARE, A CORPORATION OF DELAWARE.

## COMPOSITION FOR DETONATORS.

No Drawing.

Application filed October 16, 1922. Serial No. 594,979.

To all whom it may concern:

Be it known that BENNETT GROTTA, citizen of the United States, residing at Tamaqua, in the county of Schuylkill and State of Pennsylvania, has invented certain new and useful Improvements in Compositions for Detonators, of which the following is a specification.

This invention relates to a blasting cap 10 composition and this application is a continuation in part of my application Serial Number 517,661, filed November 25, 1921. Patent No. 1,439,099 of December 19, 1922.

The application above referred to covers 15 broadly the use of mercurous azide and fulminate of mercury as a blasting cap or detonator composition and also covers the use of these ingredients in combination with an oxidizing agent, such as potassium chlorate 20 and further covers the use of the foregoing in combination with a suitable secondary charge, such as T. N. T.

The present continuing application is 25 closely related to the foregoing and is intended to cover:

(a) Certain specific proportions of the ingredients found upon extensive investigation to give highly efficient results in an economical way; and

(b) Certain claims originally presented in the above named parent application and cancelled therefrom under the requirement of division and which claims relate to a specific type of secondary charge.

U. S. Patents 904,289 of November 17, 1908 and 1,128,394 of February 16, 1915 both issued to L. Wohler, disclose the use of an azide in a detonating compound but the particular metal disclosed by the aforesaid patents is lead azide and not mercurous azide as set forth herein. There are certain technical reasons why mercurous azide is much more efficient for use in the connection stated than lead azide, particularly when the metal azide is to be mixed with fulminate of mercury. Among these reasons may be mentioned the following:

Different metals or alloys which are suitable for detonator casings or shells in most cases react oppositely with fulminate of mercury and lead azide so that as a rule a shell material which is satisfactory for one compound is highly unsatisfactory for the other. For instance, fulminate of mercury can be used in copper shells, but cannot be used

in zinc or aluminum shells because, due to electrolytic or chemical action, it affects a rapid corrosion of the zinc or aluminum shells, similarly, lead azide may be used in aluminum shells, but cannot be used in copper 60 shells because, in contact with copper, lead azide forms a dangerously sensitive copper azide. Thus it is evident that a mixture of these two compounds cannot be used in shells made of certain non-sparking metals, 65 such as copper and aluminum, because the metal which would be suitable for the one compound would be attacked by the other.

The above explanation is fully confirmed by experiments and by the fact that there is 70 now being marketed a tetryl detonator, primed with lead azide, which, in turn, is covered with a third charge of an easily ignitable substance, other than fulminate of mercury, all of which is contained in an 75 aluminum shell. Therefore, it would appear that all hope of utilizing a mere mixture of fulminate and an azide has been abandoned. The foregoing difficulties do not exist with respect to the mercurous salt 80 of hydrazoic acid employed by me which salt may be mixed with fulminate of mercury, with or without the addition of potassium chlorate and charged into ordinary detonator shells without deterioration of the 85 latter.

Although the mercury salts of hydrazoic acid have been considered too dangerous to have practical importance I have found that the mercurous compound, in contradistinction to the mercuric azide, can be made by methods which will produce a comparatively safe product. Mercurous azide is admirably suited for admixture with mercury fulminate because, in the first place, 90 both compounds being salts of the same metal may be mixed without danger of chemical action, and in the second place, there is no appreciable action between such a mixture and shells which would be suitable for fulminate detonators. Throughout 95 extensive experimentation I have found that the mercurous compound, in contradistinction to lead azide, does not form the super sensitive copper azide. Even in a moist atmosphere of carbon dioxide, copper is not appreciably attacked by mercurous azide, while, under similar conditions, lead azide very rapidly gives rise to the dangerous copper compound. The secret of this chemi- 100 105 110

cal inactivity of mercurous azide has two possible explanations, either of which may be dependent on the other.

1. The comparative positions of the metals involved, in the electro-motive series.

2. The comparative solubilities of mercurous azide and lead azide in water.

It is a well known fact that the mutual reactivity of different salts and metals is largely dependent on the positions of the metals involved in the electro-motive series, with respect to hydrogen. In general the wider the gap between two metals, the more rapid will be the reaction. The following table of specific electrode potentials indicates a positive potential value for both aluminum and lead and negative values for copper and mercury. This is in accord with the fact that mixtures of lead azide and fulminate of mercury cannot be used in either copper or aluminum shells.

| Metals.  | Electrode potentials. |
|----------|-----------------------|
| Aluminum | +1.040*               |
| Lead     | +0.12**               |
| Copper   | -0.51                 |
| Mercury  | -0.80                 |

\*Neumann, Zeitshrift fur Physik, chemie, 14, 229.

\*\*Noyes and Sherrill, Principles of Chemistry, p. 164.

It is also a well known fact that no metal can displace another metal from a salt unless water or other solvent be present. Therefore the relative solubilities of two difficultly soluble salts should furnish an index of their comparative reactivity with respect to a metal. I have found by actual experiments that mercurous azide is soluble in water at ordinary temperature to the extent of 0.03 grams per liter, while lead azide, under the same conditions, is soluble to the extent of 0.38 grams per liter. A small amount of water is almost unavoidably present in a detonator charge, remaining from a previously wet condition of the ingredients, or from being supplied from the moisture in the air, or both. The fact that lead azide is more than twelve times as soluble as mercurous azide is also in accord with the much greater tendency of lead azide to have its metal displaced by certain other metals, such as copper.

The action of carbonic acid must also be considered. Carbon dioxide is present in the atmosphere. In combination with water it forms carbonic acid, which may act upon the azide with the liberation of the highly volatile hydrazoic acid, which in turn may act upon the copper of the shell, with the formation of the dangerous copper azide. The above figures show that mercurous azide is almost insoluble. Thorough and

exhaustive tests in an atmosphere of carbon dioxide and moisture have shown that copper or gilding metals shells with mercurous azide do not form this dangerous compound in a detectable amount, even over a long period of time. Lead azide, on the other hand, under the same comparative conditions quickly forms a deposit of this supersensitive compound.

Further, under the influences of moisture and carbon dioxide, lead azide may be converted to a non-explosive mass, while, under the same conditions, mercurous azide is not noticeably affected. It is well known that ordinary air contains moisture and carbon dioxide and that mine air often contains even greater amounts.

In addition to being wholly practical from a standpoint of stability, I have found that from a standpoint of detonating efficiency, the admixtures of small quantities of mercurous azide with fulminate of mercury, produces most gratifying results. By extensive experimentation I have also found that the advantageous effects of such mixtures hold equally true when the mixtures include suitable proportions of potassium chlorate. The addition of potassium chlorate to the primary detonating composition in detonators is a well known and common procedure. These advantages may be summarized as follows:

1. The brisance or detonating value is greatly increased. The inner capsule, which is essential in a mercury fulminate-tetryl detonator, may be dispensed with, and a smaller priming charge used effectively.

2. Such mixtures are practically unaffected by moisture, whereas mercury fulminate or mercury fulminate-potassium chlorate alone are easily and quickly made ineffective by moisture.

3. Detonators charged with such mixtures are unimpaired by pressures at which fulminate of mercury or fulminate of mercury-potassium chlorate mixtures become "dead pressed."

4. Such mixtures retain the same property of ease of ignition as does straight mercury fulminate, the flash point of various mixtures being practically identical with that of fulminate of mercury.

The proportions employed in the charging of a blasting cap are as follows: A base charge consisting of 0.4 of a gram of tetryl and a 0.4 gram priming charge, made up of 60% fulminate of mercury, 20% mercurous azide and 20% chlorate of potassium.

While I prefer to employ tetryl as the base charge the invention is not necessarily limited thereto, since the proportions recited for the priming charge are of importance and advantageous in connection with various kinds of base or secondary charges among which may be mentioned tetranitro-

aniline, nitro-starch, hexanitrodiphenylamine, T. N. T. or cyclotrimethylenetrinitramine.

Having described my invention what I claim is:

1. A detonator charge containing fulminate of mercury, mercurous azide and tetryl.
  2. A detonator charge containing fulminate of mercury, mercurous azide, potassium chlorate and tetryl.
  3. A detonator charge comprising a priming charge made up of 60% of fulminate of mercury, 20% mercurous azide and 20% chlorate of potassium.
  4. A detonator charge comprising a base
- charge of tetryl and a priming charge made up of 60% of fulminate of mercury, 20% mercurous azide and 20% chlorate of potassium.
5. A detonator charge comprising a base 20 charge of 0.4 gram of tetryl and a 0.4 gram priming charge made up of 60% fulminate of mercury, 20% mercurous azide and 20% chlorate of potassium.

In testimony whereof he affixes his signature in the presence of two witnesses.

BENNETT GROTTA.

Witnesses:

R. L. HILL,  
H. N. FINN.